

# United States Patent Office

3,007,872

Patented Nov. 7, 1961

1

3,007,872

MINERAL LUBRICATING OIL COMPOSITIONS  
Arthur Donald Shellard, Wrexham, North Wales, Charles Norman Thompson, Widnes, Donald Keith Gilmour, Upton Park, Chester, and Robert James Morris, Wallasey, England, assignors to Shell Oil Company, a corporation of Delaware  
No Drawing. Filed Dec. 5, 1957, Ser. No. 700,737  
3 Claims. (Cl. 252—48.6)

This invention relates to an improved process for improving the properties of hydrocarbon lubricating oils. More particularly it relates to a process for the preparation of improved lubricating oil additives and to hydrocarbon lubricating oils containing added amounts of such additives and having enhanced properties.

An important factor affecting the ability of a mineral lubricating oil to lubricate effectively various machine elements such as in internal combustion engines, gears, etc., is the spreading pressure of the mineral lubricating oil on the solid surfaces involved.

It has now been discovered that the spreading pressure of hydrocarbon lubricating oils on solid surfaces can be increased easily and economically without any adverse effects on the chemical or physical properties of the oil by treating such lubricating oils containing at least 5% naturally occurring polyaromatic and heterocyclic materials therein and at least 0.1% sulfur with a small amount of a per(carboxylic) acid. More particularly it has been found that when certain high sulfur-content mineral oil fractions, identified more fully hereinafter, are treated with an organic per(carboxylic) acid a product is obtained which has a very high spreading pressure on solid surfaces. The product, blended in a hydrocarbon lubricating oil, raises the spreading pressure of the oil on solid surfaces. Moreover, in the treatment of the high sulfur-content fraction with the peracid, a substantial portion of the peracid in relation to the oil fraction may be used. Since the treated mineral oil fraction is normally required to be added to the base hydrocarbon lubricating oil in only a small proportion, this use of a substantial proportion of peracid in the treatment of the mineral oil fraction does not impair the other properties of the finished lubricating oil and does not prove to be uneconomic. Moreover, the sulfur content of the mineral oil fraction is not substantially changed by the treatment.

The certain high sulfur-content mineral lubricating oil fractions, referred to are either, (1) a mineral lubricating oil aromatic extract containing at least 0.2% sulfur and more than 5% polyaromatic and heterocyclic materials or (2) a high sulfur-content (at least 1%) content mineral oil having an initial boiling point of at least 300° C. and a viscosity-gravity constant of at least 0.9. The viscosity gravity constant is defined by the relation between the viscosity and specific gravity of the oil as follows:

$$VGC = \frac{10G - 1.0792 \log (V-38)}{10 - \log (V-38)}$$

where  $G$ =specific gravity of the mineral at 60° F. and  $V$ =viscosity of the mineral oil at 100° F. in Saybolt Universal units.

It has already been proposed to reduce the sulfur content of hydrocarbons such as gasoline and the like by treating such hydrocarbons with peracids which contain the group  $—O—OH$  and therefore, by hydrolysis, will form hydrogen peroxide, for example, peracids such as peracetic or perpropionic acids. Such prior proposals were designed primarily for sweetening gasoline or kerosene by removing sulfur compounds from them, and involve

2

the use of substantial proportions of peracids, and were not concerned with improving lubricating oils or with the manufacture of lubricating oil additives. On the other hand, in the process of the present invention, only a small proportion, not more than 1.5% by weight, of the peracid is used when treating the lubricating oil to improve the oil directly, or a larger amount of peracid is used when applying it to the treatment of certain oil fractions as already defined. When the treatment is practiced in accordance with the present invention there is little, if any, reduction in the sulfur content of the treated oil. Furthermore, the sulfur-containing compounds are converted into more effective lubricating oil components having the same number of sulfur atoms per molecule, but in different chemical combination, and containing a smaller atomic proportion of carbon while maintaining it at a large number per molecule, thereby providing modified compounds in which the sulfur atoms are in more effective chemical combination and oxidatively unstable organic groups are removed to produce a more stable product.

The present process may be applied to any type of mineral lubricating oil having an initial boiling point of about 300° C., and which contain at least 0.1%, and preferably above 0.2%, even better at least 1% sulfur, and at least 5% polyaromatic and heterocyclic materials. The oil may be derived from a naphthenic, paraffinic or asphaltic crude petroleum. Generally, when applied as a minor treatment with not over 1.5% peracid, it can be applied to mineral lubricating oils of this type which have been refined by one of the conventional refining treatments, such as sulfuric acid or oleum treatment, earth or lime treatment, or solvent extraction with a selective solvent for the aromatic components. It is applicable to paraffinic-type lubricating oil, e.g., lubricating oils derived from Pennsylvania, Mid-Continent and West Texas crude oils and lubricating oils derived from other sources which may have had their paraffinicity increased by solvent extraction with selective solvents for the aromatic components.

Oil additives can be prepared by the process of the invention by treating already defined fractions (1) and (2), with peracids to form oil-soluble high molecular weight sulfones and sulfoxides and mixtures thereof having an oil solubility of at least 1% and being thermally stable up to about 250° C., and having a molecular weight between about 300 and about 1000.

The aromatic extract oil fraction (1) is one containing sulfur and may be the whole of an aromatic extract or one or more portions thereof, such as a distillate fraction or a fraction isolated by an absorption process. Such aromatic extracts can be obtained by any suitable means. The extraction of mineral oils with solvents capable of selectively extracting the aromatic constituents of such oils is a well-established refinery process and any aromatic extract produced in such a process may be used as starting material for making the additives of the present invention. Typical solvents used to extract mineral oils are liquid sulfur dioxide, phenol, furfural, nitrobenzene, cresol, aniline and beta-beta-dichlor-diethyl ether. Mixtures of solvents are also used, for example, a mixture of liquid sulfur dioxide and benzene, and a mixture of propane, cresol and phenol. The mineral oil which is subjected to extraction may be any such oil having a substantial aromatic content and is preferably a mineral lubricating oil, although it may be, for example, a kerosene, gas oil or a cycle oil from a catalytic cracking process. Preferred aromatic extracts for use in this invention are those obtained by extracting a mineral lubricating oil having a viscosity of 30 to 500 seconds Redwood I at 140° F. with liquid sulfur dioxide, furfural, phenol or a mixture of propane, cresol and phenol.

The oil fraction (2) useful for preparing oil additives by the process of the invention are residual and distillate mineral oil fractions having an initial boiling point of at least 300° C., a viscosity-gravity constant (VGC) of at least 0.9 and a sulfur content of at least 1% by weight. These mineral oil fractions may be obtained from crude petroleum oils, either as residue or distillate, by distillation, e.g., distillation at atmospheric, sub-atmospheric or super-atmospheric pressure, and steam distillation. The fraction may have been partially refined, e.g., by de-asphalting with propane or butane. Preferred mineral oil fractions are those having a viscosity-gravity constant above 0.95 and those having a sulfur content between 5 and 20% by weight.

Crude petroleum oils, from which the above mineral oil fractions may be obtained, are available from a variety of sources and examples of suitable crudes are given in Table I with typical values of the sulfur content, viscosity and gravity characteristics for samples of the crude. Residual mineral oil fractions suitable for treatment according to the present may be obtained from crude sources having a sulfur content below 1% since normally on distillation the sulfur compounds concentrate in the residual fraction.

TABLE I  
*Examples of crude petroleum oils*

| Source     | Sulfur content, percent wt. | Specific gravity | Saybolt Viscosity at 100° F. seconds | Viscosity-Gravity constant |
|------------|-----------------------------|------------------|--------------------------------------|----------------------------|
| Venezuela  | 2.43                        | 0.9672           | 4,137                                | 0.91                       |
| Do.        | 2.56                        | 0.9497           | 628                                  | 0.90                       |
| Do.        | 5.29                        | 0.9965           | 4,481                                | 0.95                       |
| Do.        | 1.57                        | 0.9408           | 339                                  | 0.90                       |
| California | 0.69                        | 0.9712           | 1,900                                | 0.92                       |

A particularly preferred mineral oil fraction for treatment according to the process of the present invention is a residual mineral oil fraction derived from a semi-solid bituminous Utah crude petroleum. Typically such a fraction has the following characteristics:

Sulfur content \_\_\_\_\_ percent by weight 12.1  
Specific gravity \_\_\_\_\_ 1.007  
Viscosity in Saybolt Universal seconds at 100° F. \_\_\_\_\_ approximately 10,000  
Viscosity-gravity constant \_\_\_\_\_ 0.96

Suitable organic peracids which may be used according to the present invention are the peracids of the lower fatty acids, such as performic acid, peracetic acid, perpropionic acid and perbutyric acid, the peracids of the substituted lower fatty acids, such as monochlorperacetic acid and trichlorperacetic acid, and the peracids of the aromatic carboxylic acids, such as perbenzoic acid. Of these, performic acid and trichlorperacetic acid are the most effective, and performic acids is preferred.

The peracids may be used in the present process either as such or in *statu nascendi*. Thus, instead of treating the mineral oil or fractions thereof with a pre-formed organic peracid, the mineral lubricating oil or fractions thereof, as defined, may be treated with a mixture of the organic acid and hydrogen peroxide. When using a mixture of an organic acid and hydrogen peroxide, these reagents may be used in stoichiometric proportions but generally it is preferable to employ excess of the acid.

The treatment of the mineral oil and fractions thereof with the peracid is generally effected at ambient temperature, although any other convenient temperature, such as between 0° and 100° C., may be employed. The mineral oil or fractions thereof and the peracid should be well agitated to ensure intimate contact and, with good agitation, the reaction should be completed in a period of from 5 to 60 minutes. With large scale batches, agitation for longer periods, such as up to 2 or 4 hours, may be necessary. The proportions of peracid employed may

vary widely and depends on the oil being treated. Thus, when the oil is used rather than fraction (1) or (2), the amount of peracid used should not amount to more than 1.5% by weight of the oil. In general, a proportion of between 0.5 and 1% by weight will be used, although where only small increases in spreading pressure are required, much smaller quantities, e.g., 0.5 to 0.5% by weight, may be used. When either fraction (1) or (2) is used, the amount of peracid may be between 2 and 25%, more usually between 5 and 20%, by weight, based on the petroleum fraction treated, although where only small increases in spreading pressure are required, much smaller quantities, for example, 0.1 to 1.0% by weight, may be used.

It is sometimes convenient, for example, when the mineral oil fraction (1) or (2) is a viscous one, to dilute the mineral oil fraction with a thinner oil or solvent before treatment with the peracid. Thus, it may be diluted with thin lubricating oil, gas oil or kerosene or a solvent such as xylene, toluene or petroleum ether.

A convenient method of effecting the treatment is to mix the mineral oil or fractions thereof with the necessary proportion of an aqueous solution of hydrogen peroxide and with the organic acid. The hydrogen per-

oxide solution is conveniently used in the form in which it is readily available commercially, for example as "100-volume" hydrogen peroxide which contains 30% by weight of hydrogen peroxide. Similarly, the organic acid is conveniently used in the form in which it is available commercially. Thus, formic acid may be used as the commercial acid containing 90% by volume of H.COOH, whereas acetic acid can be used as glacial acetic acid. More dilute aqueous solutions of formic acid may be used, such as those containing 20 to 50% by volume of H.COOH. In the case of solid organic acids such as trichloracetic acid, these may be dissolved in a suitable solvent such as water or a low boiling alcohol before adding to the mineral oil or fractions thereof and hydrogen peroxide solution, or they may be dissolved or dispersed in the hydrogen peroxide solution or in the mineral oil fraction before mixing with the mineral oil fraction or hydrogen peroxide solution, respectively.

After the treatment with the peracid, the mineral oil or fractions thereof will generally require working up to remove residual acid, hydrogen peroxide and water. This may be effected by simple water washing or washing with an aqueous or alcoholic solution of an alkaline material, such as caustic soda or sodium carbonate or ammonia. The last traces of water may be removed from the treated and washed mineral oil fraction by azeotropic distillation with a volatile solvent such as benzene, toluene or xylene. Alternatively, after the treatment with the peracid, the aqueous phase is removed and a solid alkaline material, such as sodium carbonate or lime, is added to the mineral oil fraction and the mixture is filtered. A mixture of sodium carbonate and an activated earth, such as is normally used in the finishing of lubricating oils, is also a suitable solid alkaline material.

The following examples illustrate the process for preparing improved finished mineral lubricating oils of the present invention which may be used as such or blended with other lubricating oils prior to use.

#### EXAMPLE I

100 parts by weight of a solvent-refined mineral lubricating oil having a viscosity of 330 seconds Redwood I at 140° F. and a spreading pressure on steel of 7.7 dynes per centimeter was mixed with one part by volume of formic acid (90% by weight H.COOH) and 0.5 part by volume of "100-volume" hydrogen peroxide solution, and the whole stirred for 2 hours at room temperature. The treated oil was washed with water and twice with an equal volume of a 3% by weight aqueous caustic soda solution, followed by a final water wash. The finished oil had a spreading pressure on steel of 18.3 dynes per centimeter.

The analytical data on the untreated and treated oil was as follows:

|                         | Untreated                        | Treated               |
|-------------------------|----------------------------------|-----------------------|
| Carbon                  | 83.5                             | 81.2                  |
| Hydrogen                | 12.6                             | 12.8                  |
| Oxygen                  | 2.6                              | 2.8                   |
| Sulfur                  | 2.35                             | 4.0                   |
| Nitrogen                | 0.27                             | 0.10                  |
| Calc. molecular formula | $C_{47}H_{77.2}O_{1.43}N_{0.12}$ | $C_{38}H_{72}O_{8.8}$ |
| Sulfoxide, moles/kg     | 0.25                             | 0.90                  |
| Sulfone, moles/kg       | None                             | 0.10                  |

## EXAMPLE 2

A Pennsylvania 150 neutral lubricating oil which had a sulfur content of less than 0.1% by weight and a spreading pressure on steel of 15.2 dynes per centimeter was treated as in Example 1. The finished oil had a spreading pressure on steel of 27.2 dynes per centimeter.

## EXAMPLE 3

A naphthenic lubricating oil having a sulfur content of 1.0% by weight and a spreading pressure on steel of 13.1 dynes per centimeter was treated as in Example 1. The finished oil had a spreading pressure on steel of 20.4 dynes per centimeter.

## EXAMPLE 4

60 gallons of a solvent-refined mineral lubricating oil having a viscosity of 330 seconds Redwood I at 140° F., a sulfur content of 0.66% and a spreading pressure on steel of 7.8 dynes per centimeter was stirred at room temperature for 2 hours with 0.5 by volume of 100-volume hydrogen peroxide solution and 1% by volume of formic acid (90% by weight H.COOH). The oil was then mixed with 2% by weight of lime and 2% by weight of an activated earth, stirred for one hour and filtered. The filtered oil was again treated for 2 hours with 0.5% by volume of 100-volume hydrogen peroxide solution and 1% by volume of formic acid (90% by weight H.COOH) and lime and earth-treated as in the first stage and again filtered. The finished oil had a sulfur content of 0.65% and a spreading pressure on steel of 18.3 dynes per centimeter.

## EXAMPLE 5

100 parts by weight of a solvent-refined mineral lubricating oil having a viscosity of 330 seconds Redwood I at 140° F., and a spreading pressure on steel of 7.8 dynes per centimeter were stirred for 2 hours with 1 part by volume of 100-volume hydrogen peroxide solution and 1 part by volume of formic acid (90% by weight H.COOH) at room temperature. The mixture was stirred with 1% by weight of an activated earth and 1% by weight of lime for 30 minutes and then filtered. The finished oil had a spreading pressure on steel of 19.1.

## EXAMPLE 6

100 parts by weight of the solvent-refined mineral lubricating oil used as starting material in Example 5 were stirred for 2 hours with 1 part by volume of 100-volume hydrogen peroxide solution and 1.25 parts by volume of glacial acetic acid. The mixture was then stirred with 2% by weight of activated earth and 2% by weight of lime for 30 minutes and then filtered. The finished oil had a spreading pressure on steel of 14.1 dynes per centimeter.

## EXAMPLE 7

Example 6 was repeated using 1.5 parts by volume of propionic acid in place of the acetic acid. The finished oil had a spreading pressure on steel of 16.0 dynes per centimeter.

## EXAMPLE 8

Example 6 was repeated using 2 parts by volume of butyric acid in place of the acetic acid. The finished oil had a spreading pressure on steel of 16.6 dynes per centimeter.

## EXAMPLE 9

Example 6 was repeated using 0.25 gram mols of mono-

chloracetic acid in place of the acetic acid. The finished oil had a spreading pressure on steel of 16.5 dynes per centimeter.

## EXAMPLE 10

5 Example 6 was repeated using 0.25 gram mols of trichloracetic acid in place of the acetic acid. The finished oil had a spreading pressure on steel of 17.6 dynes per centimeter.

## EXAMPLE 11

10 The process of Example 6 was applied to the treatment of four different mineral lubricating oils obtained as raffinates from the cresylic acid-propane duosol extraction of mineral lubricating oil fractions. The viscosities of the oils, their initial spreading pressure on steel and their spreading pressure on steel after being subjected to the process are set out in Table II:

TABLE II

|     | Viscosity in seconds Redwood I at 140° F. | Spreading pressure on steel of untreated oil, dynes/cm. | Spreading pressure on steel of treated oil, dynes/cm. |
|-----|-------------------------------------------|---------------------------------------------------------|-------------------------------------------------------|
| 25  |                                           | 7.9                                                     | 20.3                                                  |
| 65  |                                           | 8.7                                                     | 18.8                                                  |
| 220 |                                           | 6.1                                                     | 17.3                                                  |
| 440 |                                           | 8.0                                                     | 17.1                                                  |
| 650 |                                           |                                                         |                                                       |

## EXAMPLE 12

30 The process of Example 5 was repeated on six different mineral lubricating oils obtained as raffinates from the furfural extraction of mineral lubricating oil fractions. The viscosity of the treated oils and their spreading pressure on steel before and after treatment is set out in Table III.

TABLE III

|     | Viscosity in seconds Redwood I at 140° F. | Spreading pressure on steel of untreated oil, dynes/cm. | Spreading pressure on steel of treated oil, dynes/cm. |
|-----|-------------------------------------------|---------------------------------------------------------|-------------------------------------------------------|
| 40  |                                           |                                                         |                                                       |
| 65  |                                           | 9.3                                                     | 22.8                                                  |
| 160 |                                           | 8.7                                                     | 25.5                                                  |
| 260 |                                           | 10.3                                                    | 22.4                                                  |
| 45  |                                           |                                                         |                                                       |
| 55  |                                           | 10.3                                                    | 24.4                                                  |
| 160 |                                           | 8.4                                                     | 23.4                                                  |
| 650 |                                           | 4.8                                                     | 21.5                                                  |

50 The analytical data on the untreated and treated oil (65 second viscosity in Redwood I at 140° F.) was as follows:

|                         | Untreated                          | Treated                          |
|-------------------------|------------------------------------|----------------------------------|
| Carbon                  | 82.1                               | 77.0                             |
| Hydrogen                | 11.5                               | 12.3                             |
| Oxygen                  | 3.8                                | 4.7                              |
| Sulfur                  | 3.9                                | 6.8                              |
| Nitrogen                | <0.01                              | <0.01                            |
| Calc. molecular formula | $C_{39.0}H_{59.5}O_{1.05}S_{0.54}$ | $C_{23}H_{34.7}O_{1.35}S_{1.00}$ |
| Sulfoxide, moles/kg     | 0.2                                | 1.65                             |
| Sulfone, moles/kg       | None                               | 0.15                             |

60 The following examples illustrate the process of preparing lubricating oil additives from aromatic extracts (1).

## EXAMPLE 13

65 The aromatic extract used in this example was prepared by extracting a Venezuelan naphthenic spindle oil distillate having a viscosity of 45 seconds Redwood I at 140° F. with liquid sulfur dioxide and removing the sulfur dioxide from the extract. This aromatic extract had a viscosity of 51 seconds Redwood I at 140° F. 100 parts by weight of this aromatic extract were mixed with 10 parts by volume of formic acid (90% by weight H.COOH) and 5 parts by volume of 100-volume hydrogen peroxide solution and the whole stirred for 3 hours at 20° C. The treated oil was washed with water until

neutral and the oil finally dried by azeotropic distillation with benzene.

To a mineral lubricating oil which had been refined by the Duosol process and which had a viscosity of 330 seconds Redwood I at 140° F. and a spreading pressure on steel of 9 dynes per centimeter was added 1% by weight of the peracid treated aromatic extract. The resulting lubricating oil had a spreading pressure on steel of 13.3 dynes per centimeter. When 4% by weight of the treated aromatic extract was used, the resulting lubricating oil had a spreading pressure on steel of 19.2 dynes per centimeter, and, when 8% of the treated aromatic extract was used, the resulting oil had a spreading pressure on steel of 23.8 dynes per centimeter (Composition 13).

#### EXAMPLE 14

50 parts by weight of the performic acid-treated aromatic extract prepared as in Example 13 were mixed with 10 parts by volume of formic acid (90% by weight H.COOH) and parts by volume of 100-volume hydrogen peroxide solution and the whole stirred for 3 hours at 20° C. The product was washed with water until neutral and the treated oil dried by azeotropic distillation with benzene.

When 4% by weight of this product was added to the mineral lubricating oil referred to in Example 13, the resulting lubricating oil had a spreading pressure on steel of 23.6 dynes per centimeter and, when 8% by weight of the product was used, the resulting lubricating oil had a spreading pressure on steel of 25.1 dynes per centimeter (Composition 14).

#### EXAMPLE 15

200 parts by weight of the aromatic extract referred to in Example 13 were mixed with 8 parts by volume of formic acid (90% by weight H.COOH) and 8 parts by volume of 100-volume hydrogen peroxide solution and stirred for 2 hours at room temperature. A further 8 parts by volume of the formic acid and of the hydrogen peroxide solution were then added and stirring continued for a further 2 hours. 8 parts by volume of the hydrogen peroxide solution were then added and stirring continued for 2 hours and then a further 8 parts by volume of a hydrogen peroxide were added and the stirring continued again for 2 hours. The aqueous layer was separated off, and the oil was washed with water until neutral and the dried by azeotropic distillation with benzene.

When 2% by weight of the above product was blended into the mineral lubricating oil described in Example 13, the spreading pressure on steel of the resulting lubricating oil was 19.6 dynes per centimeter (Composition 15).

#### EXAMPLE 16

200 parts by weight of the aromatic extract referred to in Example 13 were mixed with 8 parts by volume of formic acid (90% by weight H.COOH) and 8 parts by volume of 100-volume hydrogen peroxide solution and stirred for one hour at 80° C. A further 8 parts by volume of the formic acid and of the hydrogen peroxide solution were then added and stirring continued for a further hour at 80° C. 8 parts by volume of the hydrogen peroxide solution were then added and stirring continued for 2 hours at 80° C. The aqueous layer was separated off and the oil washed with water until neutral. The product was then dried by azeotropic distillation with benzene.

When 2% by weight of the above product was blended into the mineral lubricating oil referred to in Example 13, the spreading pressure on steel of the resulting lubricating oil was 20.2 dynes per centimeter (Composition 16).

#### EXAMPLE 17

Example 16 was repeated up to the point where the aqueous layer was separated off from the treated aro-

matic extract. After the separation of this aqueous layer, the treated aromatic extract was mixed with solid sodium carbonate in a small excess over the quantity necessary to neutralize the excess acidity in the aromatic extract, together with 1% by weight of activated earth. The mixture was stirred and filtered.

To a mineral lubricating oil having a viscosity of 330 seconds Redwood I at 140° F. and a spreading pressure on steel of 8 dynes per centimeter, there was added 2% by weight of the resulting performic acid treated aromatic extract. The finished lubricating oil had a spreading pressure on steel of 19.2 dynes per centimeter (Composition 17).

#### EXAMPLE 18

15 The aromatic extract used in this example was obtained by extracting a Venezuelan neutral naphthenic lubricating oil distillate having a viscosity of 230 seconds Redwood I at 140° F. with liquid sulfur dioxide and removing the latter from the extract. This aromatic extract 20 had a viscosity of 350 seconds Redwood I at 140° F. 100 parts by weight of this extract were diluted with 50 parts by weight of a light petroleum spirit (boiling range 60° to 80° C.) in order to reduce its viscosity. The 25 diluted extract was mixed with 10 parts by volume of formic acid (90% by weight H.COOH) and 5 parts by volume of 100-volume hydrogen peroxide solution and the whole stirred for 3 hours at room temperature. It was then washed with water until neutral and the petroleum spirit and water were removed by distillation under vacuum.

When 1% by weight of the above product was added to the mineral lubricating oil referred to in Example 13, the resulting lubricating oil had a spreading pressure on steel of 16.9 dynes per centimeter. When 4% of the product was so added, the resulting lubricating oil had a spreading pressure on steel of 19 dynes per centimeter (Composition 18).

#### EXAMPLE 19

40 A heavy cycle oil from a fluidized catalytic cracking process, which cycle oil had a viscosity of 67 seconds Redwood I at 100° F., was extracted with furfural and the extract phase distilled. The fraction boiling from 200° to 250° C. at 20 mm. of mercury pressure was taken as the aromatic extract for this example.

45 10 parts by weight of this aromatic extract were mixed with 5 parts by volume of formic acid (90% by weight H.COOH) and 5 parts by volume 100-volume hydrogen peroxide solution and the whole stirred for 2 hours at room temperature. A further 5 parts by volume of each of the formic acid and the hydrogen peroxide solution were then added and the mixture stirred for a further 4 hours. The mixture was then washed with water until neutral. An equal volume of benzene was added 50 and the extract/benzene blend was added to a mineral lubricating oil having a viscosity of 330 seconds Redwood I at 140° F. and a spreading pressure on steel of 18 dynes per centimeter in such a proportion that the finished oil would contain 2% by weight of the treated aromatic extract. The benzene was stripped off from the resulting mixture together with residual water and the finished lubricating oil was found to have a spreading pressure on steel of 25 dynes per centimeter.

#### EXAMPLE 20

55 A sulfuric acid treated transformer oil extract fraction was treated with performic acid in two stages using each time 5 ml. of 90% formic acid and 5 ml. of 100-volume hydrogen peroxide per 100 grams of extract. The 60 spreading pressure on steel of a 3% blend of the treated extract in a mineral lubricating oil having a viscosity of 330 seconds Redwood I at 140° F. was 19.6 dynes/cm. (Composition 20) compared to 10.5 dynes/cm. for a 3% blend of the untreated extract and 7.6 dynes/cm. for the base oil.

Analytical data and infrared spectroscopic estimations of sulfoxide and sulfone concentrations for the treated and untreated extracts were:

|                    | Untreated Extract | Treated Extract |
|--------------------|-------------------|-----------------|
| C, wt. percent     | 86.4              | 85.4            |
| H, wt. percent     | 9.8               | 9.7             |
| O, wt. percent     | 0.6               | 2.2             |
| S, wt. percent     | 3.3               | 2.9             |
| Sulfoxide, mole/kg | 0.10              | 0.35            |
| Sulfone, mole/kg   | Trace             | 0.30            |

The increase in oxygen content (measured directly) during treatment is 1.0/gram-atom per kilogram; thus 85% of the oxygen added by performic acid treatment has entered into sulfone and sulfoxide linkages.

The following examples illustrate the process of making lube oil additives from high sulfur-content mineral oil fractions (2) having an initial boiling point of at least 300° C. and a viscosity-gravity constant (V6C) of at least 0.9.

#### EXAMPLE 21

200 parts by weight of a residual mineral oil fraction derived from a semi-solid bituminous Utah crude petroleum which fraction had an initial boiling point of 370° C., a sulfur content of 12% and a viscosity-gravity constant of 0.96, were mixed with 200 parts by weight of a hydrocarbon oil having a boiling point between 60° and 80° C. and agitated for 4 hours at 20° C. with 8 parts by volume of 100-volume hydrogen peroxide and 16 parts by volume of formic acid (90% HCOOH). The treated mineral oil fraction was washed with water until neutral and finally dried by azeotropic distillation with benzene. The sulfur content of the treated mineral oil fraction was 12%.

The treated mineral oil fraction was added in the proportion of 1% by weight to a mineral lubricating oil, which had been refined by the Duosol process and had a viscosity of 330 seconds Redwood I at 140° F. and a spreading pressure on steel of 9 dynes per centimeter. The spreading pressure on steel of the lubricating oil after addition of the treated mineral oil fraction was 23 dynes per centimeter (Composition 21).

#### EXAMPLE 22

100 parts by weight of a mixture comprising a residual mineral oil fraction derived from a semi-solid bituminous Utah crude petroleum, having a sulfur content of 12%. a viscosity-gravity constant of 0.96 and an initial boiling point of 350° C., and a mineral lubricating oil having a viscosity of 60 seconds Redwood I at 140° F. in which the sulfur content of the resulting mixture was 1.8%, was treated at 90° C. for one hour with a mixture of 5 parts by volume of 100-volume hydrogen peroxide solution and 10 parts by volume of formic acid (90% HCOOH). A further 5 parts by volume of hydrogen peroxide and 10 parts by volume of formic acid were then added to the mixture and agitated for a further period of one hour. The resulting liquid was mixed with another 5 parts by volume of hydrogen peroxide and 10 parts by volume of formic acid and agitated again for an hour. The treated hydrocarbon oil mixture was washed with water and dried by azeotropic distillation with benzene.

To a mineral lubricating oil which had been refined by the Duosol process and having a viscosity of 330 seconds Redwood I at 140° F. and a spreading pressure on steel of 9 dynes per centimeter was added 1% of the above treated Utanol mixture and the resulting lubricating oil had a spreading pressure on steel of 11.0 dynes per centimeter. When 7% by weight of the treated mixture was added to the mineral lubricating oil the resulting lubricating oil had a spreading pressure of 21 dynes per centimeter (Composition 22).

In the above examples the active components present in the oils after the peracid treatment were separated

by elution chromatography on silica gel and on infrared spectroscopic inspection were found to be sulfoxides and sulfones, predominantly sulfoxides, containing a thio-phenic structure such as hydrogenated thiophenic, benzo-thiophenic and dibenzothiophenic structures and having a molecular weight in the range of 300 to 1000.

In addition to improving the spreading pressure of lubricating oils and oil compositions in the manner described, their oxidation stability and cleanliness properties are also greatly improved. To show that peracid treated mineral lubricating oils and oil compositions containing peracid treated petroleum fractions of such are more stable and resistant to sludging and lacquer formation than untreated oils, the oils and oil compositions identified below were subjected to the Dornte Oxidation Test (catalyst, Cu 10 p.p.m. and Fe 10 p.p.m., temperature 150° C.) and the Hercules 100-hour cycling single-cylinder engine test and the results were as follows.

Mineral lubricating oils of examples such as Examples 1, or 4 to 12 when untreated had a Dornte time for uptake of 1500 ml. of oxygen per 100 g. oil of about 100 minutes, whereas the peracid treated oils of Examples 1 or 4 to 12 gave values of above 140. The Hercules Engine overall cleanliness rating (100=perfect, 0=heavy sludge) of the untreated oils of Examples 1 and 4 to 12 were around 56 whereas for the peracid treated oils of Examples 1 and 4 to 12 gave a rating of around 74. Examples 14 to 22 when untreated and compositions 13, 14, 15, 16, 17, 18 and 20 containing no peracid treated petroleum fractions in the Dornte and Hercules engine tests indicate no improvement in spreading pressure or engine cleanliness whereas the corresponding peracid treated oils (Examples 14-22) or oils containing peracid treated petroleum fractions (Compositions B-18 and 20) indicate improvement in oxidation stability, engine cleanliness and increase in spreading pressure.

If low molecular weight sulfones having an oil solubility of less than 1% such as diamyl or dicyclohexyl sulfones or sulfoxides or sulfur-free oxidized aromatics (oxidized amyl naphthalene) are used in Compositions 13-18 or 20 for the peracid treated aromatic extract or peracid treated residual oil fractions, the spreading pressure of such compositions remain the same as that of the base oil in the Dornte oxidation test and Hercules engine test the results are the same as for the base oil, namely about 100 (Dornte oxidation test) and 56 for the overall cleanliness rating in the Hercules engine test.

Hydrocarbon lubricating oils produced in accordance with the present invention may be blended with fatty oils, such a rape seed oil and lard oil, or with synthetic lubricating oils or mixtures of synthetic lubricating oils and fatty oils. Synthetic lubricating oils which can be blended with hydrocarbon lubricating oils which contain treated mineral oil fractions according to this invention, include those produced by polymerization of olefins or by the alkylation of aromatic hydrocarbons with olefins or alkyl halides in the presence of a Friedel-Crafts catalyst, organic ester lubricating oils, such as the dialkyl esters of dicarboxylic acids, for example, di(2-ethylhexyl) sebacate or adipate, and the alkyl or alkaryl esters of inorganic acids, for example, trioctyl or tricresyl phosphate and tetraoctyl silicate, polymers or copolymers of polyalkylene glycols and the esters and ethers thereof and polyorganosiloxanes.

We claim as our invention:

1. A mineral lubricating oil having incorporated therein from about 1% to about 8% by weight sufficient to stabilize the oil and increase the spreading pressure of the oil, of an additive prepared by contacting a petroleum fraction selected from the group consisting of (1) an oxygen and sulfur containing aromatic extract fraction of a mineral oil, said fraction having a sulfur content of from 0.2% to 1% and containing a minimum of 5% naturally occurring poliaromatics and hetero-

11

cyclic materials and (2) a mineral oil having an initial boiling point of about 300° C., a viscosity gravity constant of 0.9-0.95 and a sulfur content of from about 1% to about 20% with from 2% to 25% by weight of performic acid at between 0° and 100° C. for from 5 minutes to 3 hours, said treatment resulting in essentially no change in the sulfur content of the treated petroleum fraction.

2. A mineral lubricating oil having incorporated therein from about 1% to about 8% by weight sufficient to stabilize the oil and increase the spreading pressure of the oil, of an additive prepared by contacting an oxygen and sulfur-containing aromatic extract fraction of a mineral oil fraction, said fraction having a sulfur content of from about 0.2% to about 1% and containing a minimum of 5% naturally occurring polyaromatics and heterocyclic materials with from 2% to 25% by weight of performic acid at between 0° and 100° C. for from 5 minutes to 3 hours, said treatment resulting in essentially no change in the sulfur content of the treated aromatic extract fraction.

3. A mineral lubricating oil having incorporated therein from about 1% to about 8% by weight sufficient to stabilize the oil and increase the spreading pressure

12

of the oil, of an additive prepared by contacting an oxygen and sulfur-containing mineral oil fraction having an initial boiling point of at least 300° C., a viscosity gravity constant of 0.9-0.95 and a sulfur content of from about 1% to about 20% with from 2% to 25% by weight of performic acid at between 0° and 100° C. for from 5 minutes to 3 hours, said treatment resulting in essentially no change in the sulfur content of the treated aromatic extract fraction.

10

## References Cited in the file of this patent

## UNITED STATES PATENTS

|           |              |       |               |
|-----------|--------------|-------|---------------|
| 1,967,255 | Penniman     | ----- | July 24, 1934 |
| 1,972,102 | Malisoff     | ----- | Sept. 4, 1934 |
| 2,004,849 | Bretschger   | ----- | June 11, 1935 |
| 2,218,618 | McNab et al. | ----- | Oct. 22, 1940 |
| 2,749,284 | Noble        | ----- | June 5, 1956  |

## FOREIGN PATENTS

|         |        |       |              |
|---------|--------|-------|--------------|
| 758,567 | France | ----- | Nov. 3, 1933 |
|---------|--------|-------|--------------|

## OTHER REFERENCES

Kalichevsky et al.: Petroleum Refining with Chemicals, Elsevier Pub. Co., N.Y., 1956, page 23.